

## UNITED STATES PATENT OFFICE

2,250,190

## FLOTATION FROTHER

Ludwig J. Christmann, Bronxville, and David W. Jayne, Jr., Port Chester, N. Y., assignors to American Cyanamid Co., New York, N. Y., a corporation of Maine

No Drawing. Application November 5, 1937,  
Serial No. 172,898

3 Claims. (Cl. 209—166)

This invention relates to frothers and more particularly, to frothers for the froth flotation of ores.

Cresylic acids have been used with many ores as frothers in froth flotation and may be considered as standard. They are available in two boiling ranges, the lower boiling range consisting of cresols and some xylenols and the higher mainly xylenols with a few higher homologs. In spite of the fact that cresylic acids have been standard frothers for the most various types of froth flotation for so many years, they are not ideal and many synthetic frothers have been proposed, among which some, such as mixtures of aliphatic alcohols of 7-10 carbon atoms with saturated hydrocarbons as described in our Patent #2,065,053 have gone into extensive use. These synthetic frothers despite their greater efficiency are expensive and have not been successful in displacing cresylic acids for all purposes because of the relatively low price of cresylic acids until recently and their availability all over the world.

We have found that the reason why cresylic acids are not as effective frothers as could be desired lies in the fact that the length of the side chains on the phenol nucleus is too short. We have found that remarkable increases in frothing efficiencies are obtained when higher alkyl homologs or derivatives of phenol are used as frothers. The improvement is quite marked by substituting an ethyl for a methyl group and even better results are obtained with still longer alkyl chains such as propyl and butyl. Good results are obtained with longer side chains but decreasing solubilities set a limit. It is also possible to use alicyclic derivatives such as terpinyl phenols. We have found that the methyl group is not disadvantageous but it is not sufficiently long by itself, therefore, while the invention includes higher alkylated phenols which are free from methyl groups, we prefer to alkylate cresols as the raw material is somewhat cheaper and the presence of the methyl group adds somewhat to the efficiency of the resulting higher alkylated compounds as frothers.

The increase in frothing efficiency between methyl phenols and ethyl phenols is quite marked and rises rapidly to the propyl and butyl phenols such as isopropyl and secondary or tertiary butyl. Still longer hydrocarbon chains such as amyl or hexyl give good froths but the increase in efficiency over the isopropyl and butyl derivatives is too small to warrant the added price. Therefore, for practical reasons, we prefer to use the propyl or butyl derivatives such as isopropyl and tertiary or secondary butyl derivatives and these constitute the preferred embodiment of the invention.

The present invention is not concerned with

any particular method of alkylation but we have found that with the higher alcohols such as propyl and butyl and especially the secondary and tertiary alcohols, the alkylation proceeds smoothly and simply by heating with 70-80% sulfuric acid as a condensing agent. Any other method of alkylation may, of course, be used.

A typical alkylation is as follows:

10 A mixture of 1 mol of cresylic acid (boiling range, 200-215° C.) and 1 mol of isopropyl alcohol are heated at 70-75° C. with an excess of 70% sulfuric acid, the heating being maintained for three hours with good agitation. After an additional half hour of agitation, the batch is cooled and the oil layer which contains the propylated cresylic acid is separated from the aqueous phase, drawn off, washed with water, then with 10% soda ash solution, dried over anhydrous sodium sulfate and filtered. The product is a clear dark red oil having a density of 0.98 at 75° C. as compared with 1.022 for the original cresylic acid. The weight yield is about 90% of the theory and the distillation range is approximately 210-250° C.

15 It is not necessary to alkylate to the point where all of the phenols are alkylated and the invention includes frothers in which some of the phenols or cresols are not alkylated.

20 The efficiency of the frothers was tested on a lead ore having the following analysis:

|           |       | Per cent |
|-----------|-------|----------|
| 30 Pb     | ----- | 8.37     |
| Fe        | ----- | 3.10     |
| Insoluble | ----- | 10.22    |
| S         | ----- | 1.86     |

25 35 The ore was ground to 48 mesh and transferred to a Fagergren flotation machine. A lead promoter was added and one portion of the ore was treated with propylated cresylic acid and the other with the unpropylated product. The concentrates were collected, filtered, dried, weighed and assayed. In the tests, the only variable was the nature of the frother and all other conditions including amount of frother were maintained constant. The metallurgical results appear in 40 45 the following table:

| 50 | Frother                              | Amount of frother used (lbs./ton) | Concentrate      |                   | Tailing assay percent Pb |
|----|--------------------------------------|-----------------------------------|------------------|-------------------|--------------------------|
|    |                                      |                                   | Assay percent Pb | Recovery, percent |                          |
| 55 | Low-boiling cresylic acid            | 0.273                             | 70.56            | 87.36             | 1.18                     |
|    | Propylated low-boiling cresylic acid | 0.240                             | 72.03            | 97.41             | 0.25                     |

60 65 Tertiary butylated cresylic acids when tested on the same ore gave recoveries practically the same as the propylated cresylic acids but with a slightly higher grade. It will be apparent that

the alkylated cresols are markedly superior to the unalkylated cresylic acid, especially from the standpoint of recovery which is improved by 10%. The exact amount by which recoveries are improved by the use of the frothers of the present invention will vary with different ores but in all which we have tested, marked improvements are obtained by using the alkylated cresylic acids.

Terpinyl phenols gave substantially similar results to the propylated cresols but their higher cost renders them commercially less attractive although they are not excluded from the present invention.

What we claim is:

1. A method of froth flotation of lead ores 10 which comprises subjecting a pulp of lead ore to froth flotation in the presence of a flotation promoter and a frother containing a major pro-

portion of alkylated crude low boiling cresylic acid mixture, said alkyl radical being from two to five carbon atoms in length.

2. A method of froth flotation of lead ores 5 which comprises subjecting a pulp of the material to be floated to froth flotation in the presence of a flotation promoter and a frother containing a major proportion of propylated crude low boiling cresylic acid mixture.

3. A method of froth flotation of lead ores which comprises subjecting a pulp of the material to be floated to froth flotation in the presence of a flotation promoter and a frother containing a major proportion of butylated crude low boiling cresylic acid mixture.

LUDWIG J. CHRISTMANN.  
DAVID W. JAYNE, JR.